

## MAGNETIC PRODUCTS OF HIGH ALUMINUM IRON ALLOYS

Dusan Pavlovic and Karl Foster, Pittsburgh, Pa., assignors to Westinghouse Electric Corporation, East Pittsburgh, Pa., a corporation of Pennsylvania

No Drawing. Application August 16, 1957  
Serial No. 678,524

3 Claims. (Cl. 148—121)

This invention relates to a method of heat treating high aluminum-iron alloys to develop outstanding magnetic properties in the resulting products.

Aluminum-iron alloys have heretofore been annealed in dry hydrogen at temperatures of 900° to 1050° C., and the investigators have reported that the magnetic properties of the alloy were independent of the temperature of treatment. In contrast to those reported results we have found that, surprisingly, the magnetic properties of high aluminum-iron alloys annealed in hydrogen are significantly affected when the annealing temperature used is on the order of about 1200° C. Indeed, the resulting products thereby obtained have outstanding magnetic properties. That discovery forms the subject matter of our United States application Serial No. 678,539, filed August 16, 1957.

While the process of our copending patent application just referred to is entirely satisfactory as a method of producing outstanding magnetic products, it has certain aspects that are not particularly desirable from a commercial standpoint. That process is carried out in a hydrogen atmosphere. Hydrogen is readily available commercially at reasonably cost, but it constitutes a significant cost factor in the process. Moreover, where controlled atmosphere processes are practiced, equipment costs and the capital expenditures are generally higher, due to the need to use special apparatus to supply and control the atmosphere.

A temperature that may be as high as 1200° to 1300° C. (2192° to 2365° F.) also is a process variable that is not particularly desirable from a commercial standpoint. Here too, if the temperature could be materially lowered, the attractiveness of the resulting process would be enhanced.

It is a major object of the present invention to provide a method for producing aluminum-iron alloys with outstanding magnetic properties that is economical; that does not depend on hydrogen atmosphere; and that requires no special equipment for its successful utilization.

Published reports indicate that aluminum-iron alloys with as much as 11.7 percent aluminum have been air annealed. That heat treatment was stated to result in serious degradation of the magnetic properties of the alloy.

In contrast to the reported results of other investigators, we have discovered that, surprisingly, certain aluminum-iron alloys can be heat treated in air to develop outstanding magnetic properties. We have also discovered that certain compositions within the broad range of alloys, that form the subject matter of this invention, upon treatment as herein described result in magnetic properties that are on the order of the best properties heretofore obtainable. Consequently, it is apparent that we have provided an economical heat treating process by which high aluminum-iron alloys of noteworthy magnetic properties can be produced and a process whereby particular products of outstanding magnetic properties can be obtained at will.

Our invention generally is practiced by annealing a magnetic aluminum-iron alloy in air at an elevated temperature. Suitably the air anneal is carried out at a temperature of about 800° to 1000° C. and generally 5 extends for at least 30 minutes and preferably for about 1 to 5 hours. By way of example, we have air-annealed many alloys of different compositions at 900° C. for 2 hours and obtained very satisfactory results.

After annealing, the product is cooled to a temperature of about 600° to 700° C. Furnace cooling, or cooling at a rate of about 75 to 150° C. per hour, is satisfactory though a faster cooling rate such as would be experienced by air cooling also can be used if desired. The sample is cooled to a temperature approaching the ordering transformation temperature, i.e. that temperature at which the structure of the alloy changes from FeAl to Fe<sub>3</sub>Al, which normally is about 550° C. for alloys that are used in this invention. At this point, the specimen is quenched to room temperature. As is apparent, to minimize induced stresses it is desirable to quench from as low a temperature as possible. Quenching can be carried out in any manner now known that will suppress ordering transformation whereby FeAl would transform to Fe<sub>3</sub>Al. For example, the specimen 25 may be water quenched or oil quenched.

The materials to which our invention relates are magnetic aluminum-iron alloys containing about 14 to 17.5 weight percent of aluminum. Aluminum-iron alloys are non-magnetic at an aluminum content that is greater than 30 about 17.5 weight percent. Consequently, it should be understood that the upper limit, 17.5 percent, is to be construed to include the magnetic compositions and is not an absolute value. Other alloying constituents and incidental impurities may be present in varying amounts 35 provided they do not deleteriously interfere with obtaining the described improved properties in the resulting products. We have discovered that these alloys in general can be air annealed successfully to produce products with good magnetic properties. That air annealing could 40 be successful was unexpected, but it was particularly surprising to discover that at aluminum concentrations of 15 to 17 percent, the properties of the resulting product were even better than those obtained on the same alloy in a hydrogen atmosphere at the same temperature. 45 Indeed the fact that an oxygen atmosphere can be an improvement over hydrogen still cannot satisfactorily be explained.

The alloys for use in the invention can be prepared by any procedure desired. A method that we have used 50 involves vacuum melting a suitably pure iron, such as electrolytic flake iron, and then adding commercially pure aluminum having a purity on the order of 99.99 percent. The aluminum is added to the iron melt under a blanket of helium to prevent loss of the aluminum. Thereupon, the melt is cast either in a vacuum or under 55 a protective atmosphere to avoid loss of the aluminum and the uncontrolled introduction of impurities. The resulting ingot may be hot or cold rolled to the desired thickness. Generally, we roll the material to a thickness on the order of 1 to 30 mils because most commercial applications require that size; it should be understood, however, that the invention can be practiced with materials of other thicknesses.

The invention will be described further in conjunction 60 with the following representative examples. It should be understood that the details disclosed are given by way of illustration and are not intended as limiting the invention.

To demonstrate our discoveries, an aluminum-iron 65 alloy with an aluminum content of 14.7 weight percent and others with greater amounts of aluminum were prepared as follows: Electrolytic iron flake was melted in an

induction-heated, magnesium oxide crucible in a vacuum furnace at a pressure of 0.1 micron. Helium was then admitted to the furnace, and commercial aluminum bar was added to the melt. The resulting melts were cast and when the ingots had solidified, they were hot rolled at 1000° C. to 0.007 inch sheets.

Two sets of standard ring laminations were stamped from the 14.7 percent aluminum-iron (see table, below) while three sets of laminations were stamped from each sheet with an aluminum content of 15 or more percent. One set, or sample, of each composition was annealed at 900° C. for 2 hours in air; a second sample of each composition was annealed at 900° C. in dry hydrogen. The third sample of the higher compositions was annealed at 1200° C. in air for 2 hours. The annealed laminations were then furnace cooled to 600° C. Each sample was maintained at 600° C. for about 15 minutes to be sure that equilibrium was achieved and was then quenched by being immersed in water. The products were then given routine D.-C. magnetic tests to determine the coercive force, residual induction and maximum permeability. The data obtained are shown in the following table:

Table

| Run | Alloy, Percent Al | Heat Treat Atmosphere | H <sub>c</sub> <sup>1</sup><br>Oersted | B <sub>r</sub> <sup>1</sup><br>Gauss | J <sub>μ</sub> max |
|-----|-------------------|-----------------------|----------------------------------------|--------------------------------------|--------------------|
| 1.  | 14.7              | Air (900° C.)         | 0.092                                  | 3,400                                | 18,300             |
| 2.  | 14.7              | Hydrogen (900° C.)    | 0.056                                  | 3,500                                | 43,600             |
| 3.  | 15.0              | Air (900° C.)         | 0.087                                  | 2,500                                | 16,900             |
| 4.  | 15.0              | Hydrogen (900° C.)    | 0.098                                  | 2,350                                | 15,700             |
| 5.  | 15.0              | Air (1,200° C.)       | 0.087                                  | (2)                                  | (2)                |
| 6.  | 15.8              | Air (900° C.)         | 0.043                                  | 3,400                                | 54,950             |
| 7.  | 15.8              | Hydrogen (900° C.)    | 0.043                                  | 4,200                                | 73,500             |
| 8.  | 15.8              | Air (1,200° C.)       | 0.083                                  | (2)                                  | (2)                |
| 9.  | 16.2              | Air (900° C.)         | 0.031                                  | 2,750                                | 35,050             |
| 10. | 16.2              | Hydrogen (900° C.)    | 0.047                                  | 2,650                                | 30,100             |
| 11. | 16.2              | Air (1,200° C.)       | 0.049                                  | (2)                                  | (2)                |
| 12. | 16.8              | Air (900° C.)         | 0.021                                  | (2)                                  | (2)                |
| 13. | 16.8              | Hydrogen (900° C.)    | 0.029                                  | (2)                                  | (2)                |
| 14. | 16.8              | Air (1,200° C.)       | 0.037                                  | (2)                                  | (2)                |

<sup>1</sup> Taken from 100 oersted.

<sup>2</sup> Not determined.

Considering the lamination sets that were air annealed and comparing them with those that were annealed in hydrogen, it is at once apparent that alloys having an aluminum content of 14 to 17.5 percent are not degraded in their magnetic characteristics by an air treatment. Indeed, even the poorer of these properties can be classed as good and when the property is considered as a function of its cost, the values obtained take on added significance.

The data on the alloys with a 15 percent and higher aluminum content are considered to be particularly surprising. Comparing the specimens that were annealed at the same temperature but in different atmospheres (i.e. 1 vs. 2; 3 vs. 4; 6 vs. 7; 9 vs. 10; and 12 vs. 13), it can be noted that in each instance the product obtained in the air anneal was characterized by as good as or better properties (coercive force) than the hydrogen annealed product. There is no conclusive accounting for these outstanding results even after the fact.

These data also show that an anneal at 1200° C. in air can result in satisfactory properties. At 15 percent aluminum, air annealing at 1200° C. resulted in a better coercive force than in the hydrogen annealed product. On the other hand, the data of the 1200° C. air anneal point up still another anomaly of this discovery. Where-

as if the hydrogen anneal were used, a treatment at 1200° C. would result in marked improvement as compared with the results at 900° C., the use of air as the annealing atmosphere brings about just the opposite result because, as shown by the data in the table, the products obtained at 900° C. are superior to those obtained at 1200° C.

From the foregoing data and discussion it is apparent that our discoveries make it possible to produce magnetic aluminum-iron materials of noteworthy magnetic properties by a procedure that is far more economical than those known heretofore. These discoveries are particularly surprising not only because of the economical processes which they provide in face of published indications that it could not be accomplished, but also because they demonstrate another fact about aluminum-irons and their unpredictable behavior, thereby contributing to the knowledge about these alloys. These products can be substituted for the commercially available silicon-iron and nickel-iron alloys that are used in magnetic applications.

In accordance with the provisions of the patent statutes, we have explained the principle of our invention and have described what we now consider to represent its best embodiment. However, we desire to have it understood that the invention may be practiced otherwise than as specifically described.

We claim:

1. A method for providing improved magnetic properties of coercive force, remanence, and maximum permeability in an aluminum-iron alloy sheet which comprises heating in the presence of air for at least one half hour a magnetic alloy sheet consisting essentially of 14 to 17.5 weight percent of aluminum and the remainder iron at a temperature of from 800° C. to 1200° C., and then quenching the resultant annealed sheet from a temperature that is above that at which an ordering transformation occurs, wherein the structure normally changes to Fe<sub>3</sub>Al, to about room temperatures, the quenching suppressing the ordering transformation.

2. A method for providing improved magnetic properties of coercive force, remanence, and maximum permeability in an aluminum-iron alloy sheet which comprises heating a magnetic alloy sheet consisting essentially of 15 to 17 weight percent of aluminum and the remainder iron, in air at a temperature of about 800° to 1000° C. for about 1 to 5 hours, cooling the resultant annealed sheet to about 600° and then quenching the sheet to about room temperature, the quenching suppressing the ordering transformation.

3. A method according to claim 2 in which said alloy is in the form of a tape of about 5 to 30 mils in thickness.

#### References Cited in the file of this patent

#### UNITED STATES PATENTS

2,801,942 Nachman ----- Aug. 6, 1957

#### OTHER REFERENCES

60 "The Lattice Spacings of Iron-Aluminum Alloys" (Bradley and Jay), Journal of the Iron and Steel Institute, vol. 125, page 339 (1932).

65 Navord Report 4130, "The Fabrication and Properties of Alfenol Alloys (Al-Fe) Containing 10-17 Percent Aluminum," U.S. Naval Ordnance Laboratory, December 5, 1955.